

Aug. 27, 1946.

K. MARSH

2,406,554

HEATING METAL BODIES PREPARATORY TO HOT WORKING

Filed Dec. 28, 1943

Fig. 1.



Fig. 2.



INVENTOR  
Kirtland Marsh  
BY  
Howard B. Funk  
ATTORNEY

## UNITED STATES PATENT OFFICE

2,406,554

HEATING METAL BODIES PREPARATORY  
TO HOT WORKING

Kirtland Marsh, Pittsburgh, Pa., assignor to Aluminum Company of America, Pittsburgh, Pa., a corporation of Pennsylvania

Application December 28, 1943, Serial No. 515,938

6 Claims. (Cl. 263—52)

1

This invention relates to a process for heat conditioning metal bodies of considerable mass, particularly ingots, for hot working, and it is hereinafter described in connection with the treatment of ingots preparatory to hot rolling or breakdown.

To sustain a high output schedule, a common practice of processing ingots to bring them into the desired metallurgical and thermal conditions for hot rolling is carried out by the well known "soaking pit" procedure. This practice has various known deficiencies and disadvantages. Among them may be mentioned the individual handling of each ingot for removal from the heating or combustion zone, the fluctuation in pit temperature and waste of heat and fuel upon removal of the covers to expose an ingot which it is desired to remove with consequent deleterious effect on other ingots in the same heat zone or pit but not yet removed, and especially the lack of temperature equilibrium or uniformity in all parts of the ingots when they reach the mill for rolling, particularly as between the interior and exterior portions thereof.

It is among the objectives of this invention to provide a process which overcomes the foregoing and other difficulties, which eliminates individual handling of the ingots being processed, which results in maximum economy in the employment of heat and maximum conservation of heat, and by which treated or processed ingots of more uniform thermal and metallurgical conditions are produced for hot working under such predetermined schedule as may be desired and at materially lower costs. A further object of the invention is to provide an improved process whereby a large number or multiplicity of ingots may be heated up to and held at a predetermined preheating and soaking temperature above the working temperature to condition the same metallurgically, and thereafter rapidly bringing the ingots to hot working or rolling temperature, effectively establishing temperature equilibrium, throughout each ingot in readiness for rolling, and holding them indefinitely in ready condition for delivery to the mill one by one as needed. Other objects and advantages will become apparent from the following description of the invention.

By way of example, the accompanying drawing shows diagrammatically certain apparatus which may be employed in effecting the treatment of ingots in accordance with the instant invention, Fig. 1 illustrating a first furnace in which a plurality of batches of ingots are ther-

2

mally treated, and Fig. 2 illustrating a second furnace equipment in which a redistributed batch of ingots is further processed.

The nature of the preferred embodiment of the present invention may be described in general terms as including the steps of forming a multiple layer, stack or pile of the bodies or ingots to be treated with a plurality of ingots in each layer or row, introducing one or more of the piles into a soaking-preheating chamber held at a predetermined temperature above working temperature, subsequently removing a pile of heated ingots from said chamber, transferring all the ingots in the pile, in layers or in units, successively to a second furnace, and introducing the said layers of ingots into said second furnace, utilizing residual heat in the ingots while they are in the second furnace to cause equalization of temperature throughout each ingot rapidly, and advancing the ingots through the second furnace intermittently to effect discharge thereof for delivery to the mill as needed. The temperatures employed in each of the respective furnace chambers will depend upon the characteristics of the metal being treated, and specific temperatures need not be here mentioned as they are well known to the metallurgist, and for a given kind of metal the usual temperatures required to effect the desired results will be utilized. Some bodies of alloyed metals prior to initial hot working thereof require heating to a temperature above hot working temperature and soaking at that elevated temperature for a substantial length of time to improve the metallurgical characteristics, in addition to rendering the metal readily workable. Among the characteristics so improved by heating and soaking is that of structural uniformity, i. e., the heating causes some diffusion of alloy ingredients in the base metal with consequent diminution in size of brittle constituents that interfere with proper working of the bodies. The invention will be particularly advantageous for the treatment of metal bodies or ingots of such metal, aluminum alloys being a particular example.

In one mode of practicing the invention, and with reference to the drawing, a horizontal furnace 8 is provided, into the heating chamber of which the ingots are charged and there heated up to and held at a desired high temperature. The construction of this furnace may take any well known form. Preferably, it will have a heating chamber 9, spaced from the walls of the furnace and adapted for forced circulation of the furnace atmosphere by means of suitable cir-

culating fans or blowers 10, and it may be heated electrically, or by radiant tubes or in any other suitable manner, the temperature being automatically maintained at a predetermined degree in known manner. For carrying the ingots into and out of the furnace, a car 11 may be provided, on the reticulated platform of which a plurality of layers or rows of ingots assembled in piles or stacks 12 are first arranged, the car being moved by suitable means (not shown) along track 13. Piling the ingots and charging the piles horizontally enable large capacity loads to be easily handled. Either a single car with a plurality of piles thereon or a car for each pile may be used. In each pile, the ingots in each layer preferably are spaced for effective circulation around the individual ingots so that each will be uniformly heated. The layers constituting a pile preferably are cross-piled with respect to each other to provide an open and stable pile for free circulation throughout the pile. In the case of exceptionally wide ingots, spacers may be used to separate the layers thereof, as also will be the case with exceptionally long ingots stacked in parallel layers. The number of ingots in each layer and the number of layers constituting a pile will depend upon the size and spacing of the ingots. In practice, with an aluminum alloy ingot approximately 12 inches square, piles comprising five layers with five ingots in each layer and a free space of about 9 inches between ingots in the layers have successfully been employed. Piling of ingots in this manner is facilitated by initially piling the ingots received from the molds in the same way.

In the furnace 8, the batches of ingots will be brought up to a predetermined temperature above working temperature and maintained or soaked at that temperature until they are uniformly heated throughout. In the case of certain of the metal bodies heretofore mentioned, the heating will be continued until a desired degree of structural uniformity is secured, as will be readily appreciated. In either case the ingots are in condition to be removed. As distinguished from the usual "soaking pit" procedure, wherein removal of ingots is effected from the pit one by one, as required by the rolling schedule, while the others remain in the pit, with the resulting difficulty of maintaining the pit temperature uniform so that the temperature of the remaining ingots will not be impaired; according to the present invention an entire pile of the heated ingots is removed from the furnace 8.

As shown in Fig. 2, a second furnace 15 of a forced circulation type, having circulating means represented by fans 16, is provided for the reception of the entire batch or pile of ingots removed from the first furnace 8, the piled relationship of the ingots being broken down to a single layer arrangement in the second furnace 15. This furnace 15, which is operated as a holding furnace also, will be suitably heated, electrically or otherwise, and it will be provided with a suitable horizontally movable conveyor mechanism which may take the form of an endless chain type of conveyor having parallel ingot supporting chains 17 extending through the heating chamber 18. Sprockets 19 and 20, exteriorly of the discharge and the loading ends of the furnace, respectively, are provided for the chains 17, suitable power means (not shown) of a conventional type being provided to drive the chains 17, intermittent advance thereof being effected. At the discharge end of the conveyor 17, a transfer roller table 21

or the like is provided of which an ingot moved out of the furnace may be removed from the furnace conveyor and delivered to a driven roller conveyor 22, arranged in right angle relation to the holding furnace 15, by means of which the ingot thereon may be delivered to a rolling mill (not shown).

Charging of the hot ingots into the holding furnace 15 may be effected in the following manner. A complete layer of spaced ingots will be removed from the pile of heated ingots, at one time by a suitable well known grab device suspended from a crane or the like and thereby carried to the loading end of the holding furnace 15 and deposited on the conveyor chains 17 crosswise thereof. The conveyor is then advanced to move this layer of ingots into or nearly into the furnace 15, so that the next layer can be placed on the conveyor behind the first layer with substantially the same spacing therebetween as that between the ingots, and this procedure is repeated until all the layers of the pile have been charged into the holding furnace and its charging door 23 closed. Thus, in this furnace, the ingots are disposed in a single layer in spaced, side by side relationship for movement through the furnace and discharge therefrom one at a time past exit door 24 to the roller table 22 for direct and rapid delivery to the mill as needed. Of course, it will be appreciated that the conveyor mechanism and the disposition of the ingots thereon for movement through the furnace 15 are subject to variations so long as the temperature of the ingots is maintained and the ingots arranged for discharge from the furnace and delivery to the mill as required.

During transfer of the ingots in layers to the furnace 15, some drop in temperature will occur. It is desirable that the temperature to which the ingots are heated in furnace 8 be high enough to allow a full pile of ingots after withdrawal from furnace 8 to be transferred and entered into the holding furnace 15 with the average or mean temperature of the ingots when so introduced into furnace 15 to be substantially at hot working temperature. In some cases, however, where there is a relatively great temperature interval or difference between soaking and working temperatures, it may be desirable to allow some cooling to occur after removal of the bodies from the soaking furnace 8 other than that which normally occurs during transfer operations. The temperature of the holding furnace 15 need not be changed to various temperatures to accommodate individual furnace charges, but may be maintained automatically at approximately ingot working temperature.

In the holding furnace 15, the temperature of each ingot is equalized and greater temperature equality of all the ingots is effected. The furnace temperature serves to check further cooling of the surfaces of the ingots, while the residual heat in each ingot flows from the hotter interior to the exterior and brings the entire ingot to substantially a uniform temperature throughout, in readiness for working. The ingots therefore are not only maintained in ready condition for delivery one by one to the mill, but all the ingots in the holding furnace will be independent of any breakdowns or interruptions in the operation of the mill, since they may remain indefinitely in the holding furnace, thereby conserving the heat and labor employed to bring them to working condition. This is an important advantage over the prior "pit" method as it is not unusual to have

several ingots removed from the pit and in various stages of cooling down to working temperature in order to meet the mill requirements for successive ingots, and in case of interruptions the ingots removed from the pit become too cold and must be reheated. Moreover, it will be apparent that the ingots after the steps of initial thermal conditioning and charging into the holding furnace 15 are brought to a more uniform temperature throughout by reason of the equalizing action that takes place in the holding furnace prior to delivery for working, whereby the temperature of each ingot and the average or mean temperature of all the ingots are caused to be brought into a greater degree of uniformity, which manifests itself in the working operation subsequently performed. In the processing of metal bodies or ingots of certain kinds of metal, it may be advantageous to provide a non-oxidizing or inert atmosphere in the holding furnace 15 if desired.

It is preferred to discharge all of the ingots from the holding furnace 15 before introducing another batch thereinto, so that temperature conditions therein can be more readily maintained uniform and fluctuations and heat losses kept to a minimum, and crosswise ingot disposition enables a furnace and its conveyor mechanism of greatly simplified construction to be employed. Accordingly, it is preferred to provide at least an additional holding furnace 25, in all respects a duplicate of the furnace 15, arranged to discharge its ingots to the runway or roller table 22, so that uninterrupted flow of ingots to the mill can be accomplished. This furnace 25 will be charged with an entire pile or batch of ingots from the soaking-preheating furnace 8 while the mill is being supplied with ingots from the furnace 15. After the supply of ingots is exhausted from furnace 15 delivery of fully processed ingots from the furnace 25 is effected. A sufficient number of furnaces 8 will be used to supply batches of ingots to the holding furnaces 15 and 25, alternately, to meet the predetermined schedule or requirement of the mill. The discharge of ingots from the respective holding furnaces may be under control of the mill operator. Since each of the ingots as discharged from one of the holding furnaces is in required rolling condition thermally and discharge thereof is effected only as needed at the mill, there is eliminated by this invention that interdependency between the operation of the mill and the operation of associated pits extant in prior practices.

What is claimed is:

1. A process for heat conditioning cast metal bodies of an aluminum alloy and the like for initial working at a given hot working temperature comprising introducing simultaneously into a heating furnace a multiplicity of said bodies removing said bodies from said furnace simultaneously after bringing them to and maintaining them at a temperature greater than said working temperature to effect metallurgical conditioning thereof, cooling said removed bodies in air, introducing all of said removed bodies into a second furnace in side by side relation at an average temperature about equal to said working temperature to check cooling thereof, effecting equalization of the temperature of said bodies in said second furnace at substantially said working temperature, and moving said bodies through said second furnace to discharge them one at a time.

2. The method of treating cast metal alloy bodies preparatory to initial hot working at a

given hot working temperature which comprises, introducing a batch of said bodies into a furnace heated to a temperature above said working temperature, heating and soaking said bodies in said furnace, withdrawing the batch of heated bodies from said furnace, charging all the bodies constituting said batch in spaced relationship into a second furnace normally maintained substantially at said working temperature, for subsequent discharge therefrom one at a time, as needed for working, all the bodies in said second furnace being held substantially at said working temperature until discharged therefrom, and imparting intermittent movement to the said bodies in said second furnace to discharge one of them.

3. The method of treating cast metal alloy bodies preparatory to initial hot working at a given hot working temperature which comprises, introducing a batch of said bodies into a furnace heated to a temperature above said working temperature, heating and soaking said bodies in said furnace, withdrawing the batch of heated bodies from said furnace, charging all the bodies constituting said batch in spaced relationship into a second furnace normally maintained substantially at said working temperature, for subsequent discharge therefrom one at a time, as needed for working, all the bodies in said second furnace being held substantially at said working temperature until discharged therefrom, imparting intermittent movement to the said bodies in said second furnace to discharge one of them, similarly charging all the heated bodies of another batch into a third furnace identical to said second furnace during discharge of bodies from the latter, and effecting discharge of bodies from said third furnace after all the bodies have been discharged from said second furnace.

4. The method of preparing cast metal alloy bodies for initial working at a given hot working temperature which comprises, introducing a load consisting of a multiplicity of said bodies arranged in spaced piled relation into a furnace, heating said load to and soaking the same at a temperature higher than said working temperature to effect metallurgical conditioning thereof, removing the load after soaking is completed, effecting rearrangement of the said bodies of said load and introduction thereof into a second furnace without reducing the mean temperature of said bodies materially below said working temperature, equalizing the temperature of said bodies in said second furnace, prior to discharge from said second furnace, and imparting intermittent movement to said bodies in said second furnace to discharge them only as needed for working.

5. The method of preparing cast metal alloy bodies for initial working at a given hot working temperature which comprises, introducing a load consisting of a multiplicity of said bodies arranged in spaced piled relation into a furnace, heating said load to and soaking the same at a temperature higher than said working temperature to effect metallurgical conditioning thereof, removing the load after soaking is completed, effecting rearrangement of said bodies of said load and introduction thereof into a second furnace without reducing the mean temperature of said bodies materially below said working temperature, equalizing the temperature of said bodies in said second furnace primarily by the residual heat in each of them, prior to discharge from said second furnace, and imparting inter-

mittent movement to said bodies in said second furnace to discharge them only as needed for working.

6. A process for heat conditioning ingots containing alloying constituents for working at a given hot working temperature comprising arranging ingots in a pile in superposed, crossed layers with the ingots in each layer spaced from each other, introducing the pile into a heating chamber, heating the ingots to and soaking them at a temperature higher than said working tem-

perature to effect metallurgical conditioning thereof, removing the pile of ingots from said furnace after soaking is completed, removing the layers of the pile in succession, and introducing them into a second furnace in a single layer in spaced relationship, maintaining said ingots in said second furnace at a temperature substantially equal to said working temperature, and moving said ingots through said second furnace to discharge them one at a time.

KIRTLAND MARSH.